

## UNITED STATES PATENT OFFICE

WILLIAM R. CHAPIN, OF INDIANAPOLIS, INDIANA

## METAL CEMENT

No Drawing.

Application filed January 4, 1930. Serial No. 418,660.

This invention relates to cementing compounds to be used particularly in joining metals.

An object of the invention is to provide a cement which will secure perfect union between the joined metals but which will form a union less noticeable than is true with known cements. While in its use it is not to be limited to any particular metal nevertheless it has been found highly satisfactory as a cement for cementing tungsten carbide and high speed steel to a steel back or other base.

For the purposes of this compound I preferably use a mixture of silico manganese, fine steel filings and powdered borax glass. In the preparation of the product these elements are reduced to a fine powder and then thoroughly mixed to insure a strictly uniform compound throughout. While not wishing to be restricted to any strict proportion of the elements mentioned I have found the following proportions result in a highly satisfactory product, namely, 65% silico manganese, 25% fine steel filings and 10% powdered borax glass. These proportions have secured particularly good results in use with tungsten carbide, high speed steel, stellite and other metals.

In the use of my cement the parts to be cemented are placed together and are covered with approximately  $\frac{1}{2}$  of an inch of the cement. The parts are then heated to a temperature suited to the particular elements to be joined, for example, in cementing high speed steel the cementing temperature will be in the neighborhood of from 2300° to 2350° F. For stellite the temperature may be approximately 2200° to 2250° F. For tungsten carbide the cementing temperature ranges between 2175° to 2250° F. During the heating the parts are held together. After removing from the furnace the joints are pressed tightly together and any surplus compound is removed.

When large pieces are to be cemented they are first preheated to a temperature in the neighborhood of 1500° to 1600° F. They are then allowed to cool under pressure until such time as the cement has set in the joint,

then removed from the pressure and quenched. If desired the temper may be drawn afterwards to suit the work.

It will be obvious to those skilled in the art that various changes may be made in my product without departing from the spirit of the invention, and I therefore do not limit myself to those proportions named in the specification, but only as set forth in the appended claims.

Having thus fully described my said invention, what I claim as new and desire to secure by Letters Patent, is:

1. A cementing compound consisting of approximately 65% silico manganese, between 1% and 10% powdered borax glass, and the remainder fine steel filings, substantially as set forth. 65

2. A cementing compound consisting of approximately 65% silico manganese, 25% fine steel filings, and 10% powdered borax glass, substantially as set forth. 70

In witness whereof, I have hereunto set my hand at Indianapolis, Indiana, this 2nd day of January, A. D. nineteen hundred and 75 thirty.

WILLIAM R. CHAPIN.

80

85

90

95

100